

## UNITED STATES PATENT OFFICE

CYRIL J. STAUD, OF ROCHESTER, NEW YORK, AND CHARLES E. WARING, OF DAYTON, OHIO,  
ASSIGNORS TO EASTMAN KODAK COMPANY, OF ROCHESTER, NEW YORK, A CORPORATION OF NEW YORK

## PRODUCTION OF CELLULOSE NITRO-ACRYLATE

No Drawing.

Application filed December 31, 1930. Serial No. 505,960.

This invention relates to a process of preparing cellulose nitro-acrylate by nitrating the cellulose after the steps of acylation and hydrolysis, by the use of fuming nitric acid or an oxide of nitrogen after rendering the hydrolyzed dope anhydrous.

One object of our invention is to provide a method of nitration of cellulose after it has been acylated with various organic acid groups. Cellulose nitro-acrylates have been previously produced in which considerable quantities of nitrogen were present by initially nitrating the cellulose with nitric and sulphuric acids, before the acylation. Cellulose nitro-acrylates have also been produced by simultaneously nitrating and acylating the cellulose in the acylation bath by adding nitric acid shortly after the addition of the acylating agent to the pre-treated cotton linters and before a satisfactory dope has been obtained. However, no process has previously been disclosed which teaches the substantial addition of nitrogen to the cellulose subsequent to the acylation and hydrolysis of the same as is disclosed herein.

Another object of the invention is the production of a cellulose nitro-acrylate which has certain very desirable properties. The most remarkable of these characteristics is the solubility of the product of our process in a great variety of organic solvents. We have found that the mixed esters resulting from this process are soluble in acetone, chloroform, ethylene dichloride, ethyl acetate, ethyl lactate, 1.4 dioxan and pyridine.

Another object of our invention is to provide a process that can be carried out under ordinary temperature conditions. This is in contrast to the processes where simultaneous nitration and acylation are carried out, in which there is a certain element of hazard due to the use of certain nitrating agents at elevated temperatures, which may blow out apparatus and possibly injure workmen. Also these limited temperatures lead to better working conditions for the operators.

Although it has been known for a long time that the use of nitric acid in the hydrolysis

of cellulose acetate gave beneficial results, nevertheless only negligible quantities of nitrogen have thereby been introduced into the cellulose acetate, for instance, when cellulose triacetate was dissolved in 70% nitric acid, or when 70% nitric acid was added to cellulose triacetate in the acetylation mixture. By negligible amounts of nitrogen is meant less than .01%.

We have found that although 98% fuming nitric acid may be added at the close of hydrolysis in a greater concentration than usually used for nitration, nevertheless, when the dope is not dehydrated no appreciable amount of nitrogen is introduced after sixteen hours contact with the cellulose acetate dope at room temperature. We have found however that if hydrolyzed cellulose acetate, in dope form, is made substantially anhydrous, the addition of fuming nitric acid or liquid nitrogen dioxide ( $\text{NO}_2$ ) will introduce appreciable quantities of nitrogen into the cellulose ester at ordinary temperatures. If the dope after hydrolysis is to be rendered anhydrous, acetic anhydride or some other suitable dehydrating agent may be added in amounts sufficient to combine with practically all the water present to form acetic acid.

Other suitable dehydrating materials such as  $\text{P}_2\text{O}_5$ ,  $\text{B}_2\text{O}_3$ ,  $\text{SO}_3$  or fatty acid anhydrides or the like may be used. It is preferred, however, to use the anhydride of the fatty acids corresponding to the acyl group of the cellulose acylate of the dope. The term "nitrating agent" as used in this application refers to fuming nitric acid,  $\text{NO}_2$ , or its dimer  $\text{N}_2\text{O}_4$ ,  $\text{N}_2\text{O}_5$  or  $\text{N}_2\text{O}_6$ .

As an illustration of the carrying out of this process, we give the following examples:

## Example I

About 100 lbs. of acetic anhydride (85% preferred) were added to about 400 lbs. of acetic acid cellulose acetate dope, containing about 12% total solids. After thorough mixing the temperature began to rise

95

100

due to the heat liberated by the hydrolysis of the acetic anhydride. The dope was cooled to about 25° C. and about 60 lbs. of fuming nitric acid (about 98%) or liquid nitrogen dioxide was added. The temperature then started to rise, but was brought back to about room temperature by means of ice cooling. The material was then allowed to stand at 20-25° C. for fifteen to twenty hours, or until the reaction was completed, after which it was precipitated, washed and dried in the usual manner, as well known in the art. Analysis showed that the material contained about .16% nitrogen.

15                   *Example II*

About 25 lbs. of finished hydrolyzed acetic acid dope was placed in a small mixer and cooled to about 60° F. and 6-8 lbs. of acetic anhydride were added. The temperature increased to 90° F. After cooling to about 70° F., about 500 c. c. of fuming nitric acid (98% preferred) or liquid nitrogen dioxide was added in small portions. The temperature rose to about 120° F. The jacket temperature was kept around 40° F. until the inside temperature dropped to about 70 to 75° F. The outside temperature was then raised to 80° F. and held for from 5 to 8 hours, or until the reaction was complete, after which the material was precipitated, washed and dried in the usual manner. The product was found to contain about .24% nitrogen.

As the acetates are the most economical and most used of the fatty acid derivatives at the present time, the cellulose acetate dope is the preferred material. However, the dope of propionic, butyric, lauric, crotonic, etc., acids may be used. In that case the anhydride used for dehydrating may be preferably that corresponding to the acid of the dope.

It is apparent that the essential feature of our invention is the treating of a dry cellulose acylate dope which has been subjected to a hydrolysis treatment, with a nitrating agent containing an oxide of nitrogen in appreciable amount.

The solvent which is contained in the dope, the amount of hydrolysis, the dehydrating agent, temperatures and times of treatment may obviously be varied as desired the only limiting condition being that the variations are compatible with the practice of this invention. Also a mixture of the nitrating agents or of the dehydrating agents may be used where just one of these materials is called for, without affecting detrimentally the operation of this process.

60                   What we now claim as our invention and desire to secure by Letters Patent of the United States is:

1. In the process of making cellulose nitro-  
acylate the step which comprises nitrating an  
anhydrous partially de-esterified cellulose  
acylate.

2. In the process of making cellulose nitro-  
acylate the step which comprises treating a  
partially de-esterified acylated cellulose in an  
anhydrous solution with a nitrating agent.

3. In the process of making cellulose nitro- 70  
acylate, the step which comprises treating  
partially de-esterified cellulose acylate in  
solution in an anhydrous hydrolysis bath with  
a nitrating agent.

4. The step of nitrating a partially de-es- 75  
terified cellulose acylate which comprises  
treating it in an anhydrous hydrolysis bath  
with a nitrogen compound selected from the  
group consisting of fuming nitric acid,  $\text{NO}_2$   
or  $\text{N}_2\text{O}_4$ ,  $\text{N}_2\text{O}_3$  and  $\text{N}_2\text{O}_5$ .

5. The process of making cellulose nitro-  
acetate which comprises dehydrating a hy-  
drolyzed cellulose acetate dope with an acid  
anhydride and then nitrating the hydrolyzed  
cellulose acetate before it is precipitated. 80

6. The process of making cellulose nitro-  
acylate which comprises dehydrating hydro-  
lyzed cellulose acylate dope with an acid an-  
hydride selected from the group consisting  
of  $\text{P}_2\text{O}_5$ ,  $\text{SO}_3$ ,  $\text{B}_2\text{O}_3$  and acetic, propionic, 90  
butyric, lauric and crotonic anhydrides, and  
then treating the de-esterified cellulose acylate  
with a nitrating agent.

7. A process of making cellulose nitro- 95  
acylate which comprises acylating cellulose,  
hydrolyzing the cellulose acylate formed, de-  
hydrating the hydrolysis bath with an acid  
anhydride and nitrating the cellulose acylate  
contained therein.

8. The process of making cellulose nitro- 100  
acylate which comprises dehydrating a hy-  
drolyzed cellulose acylate dope with a fatty  
acid anhydride and then nitrating the dehy-  
drated cellulose acylate dope with fuming  
nitric acid.

9. The process of making cellulose nitro- 105  
acylate which comprises dehydrating a hy-  
drolyzed cellulose acylate dope with a fatty  
acid anhydride and then nitrating the dehy-  
drated cellulose acylate dope with nitrogen  
tetroxide.

10. In the process of making cellulose nitro-  
acetate, the step which comprises nitrating an  
anhydrous partially de-esterified cellulose  
acetate.

11. In the process of making cellulose nitro-  
acetate the step which comprises dehydrating  
hydrolyzed cellulose acetate dope with an acid  
anhydride.

12. In the process of making cellulose nitro- 120  
acetate the step which comprises dehydrating  
a partially de-esterified cellulose acetate dope  
with an acid anhydride selected from the  
group consisting of  $\text{P}_2\text{O}_5$ ,  $\text{SO}_3$ ,  $\text{B}_2\text{O}_3$  and  
acetic, propionic, butyric, lauric and crotonic  
anhydrides.

13. In the process of making cellulose nitro-  
acetate, the step which comprises nitrating an  
anhydrous partially de-esterified cellulose  
acetate dope with a nitrating agent selected 130

from the group consisting of fuming nitric acid,  $\text{NO}_2$  or  $\text{N}_2\text{O}_4$ ,  $\text{N}_2\text{O}_3$  and  $\text{N}_2\text{O}_5$ .

Signed at Rochester, N. Y. this 23 day of December 1930.

CYRIL J. STAUD.

5 Signed at Dayton, Ohio, this 26th day of December 1930.

CHARLES E. WARING.

10

15

20

25

30

35

40

45

50

55

60

65